

## UNITED STATES PATENT OFFICE

ADOLF HAWERLANDER, OF NEW YORK, N. Y., ASSIGNOR, BY MESNE ASSIGNMENTS, TO  
DURIUM PRODUCTS CORPORATION, A CORPORATION OF DELAWARE

## MATERIAL AND PROCESS FOR MAKING PHONOGRAPH RECORDS

No Drawing.

Application filed October 7, 1927. Serial No. 224,770.

This invention relates to sound records, and more particularly to a material and process for coating a record disk to thereafter receive the record impression. While it is adaptable for use in a so-called "laminated" type of record, it is particularly designed for coating a cardboard or other fibrous disk to form a phonograph record.

Heretofore in the manufacture of phonograph records, of the type formed from materials of dissimilar characteristics, such as laminated records and records made with cardboard cores, and as distinguished from the "solid stock" record, perhaps the most serious problem encountered has been that of a successful joinder between several unlike materials comprising the record. Such troubles have been due largely to the varying effect of temperature and moisture changes on these

unlike materials. The rate of expansion and contraction for a given change in temperature, for instance, varies in a fibrous material, such as cardboard, and in the usual kinds of coating material used to surface the cardboard and take the record impression. Again, moisture or humidity conditions in the atmosphere frequently are responsible for separating these unlike materials, or "blistering", or otherwise giving an uneven surface without sufficient durability for proper wear during normal use. These have always been most serious problems in the manufacture of a cardboard record. They are here solved for the first time through the invention of a suitable material, which eliminates these troubles, and the process of compounding such material and applying it to a special fibrous disk.

Most present-day records are made from thermoplastic material, either used throughout the record or concentrated upon its surface. Such material necessarily contains shellac, which is expensive, and has other disadvantages in use.

The present invention more especially comprises a phenol condensation product particularly adapted for use as a molding surface for phonograph records to receive and carry the tone grooves.

Another feature of the present invention resides in the special adaptability of the particular phenol condensation product herein disclosed to form an intimate bond with a fibrous or paper body for use in manufacturing phonograph records.

This coating material has many additional advantages, such as increased hardness, minimum abrasion or wear of the playing needle, and proper acoustical properties. Also, it is wholly, or almost wholly, transparent, permitting the printing of the cardboard core to be legible through the record recorded in this material which covers it.

In compounding the ingredients used in the manufacture of this coating material, a 40% solution of formaldehyde is used. The first step in the process of mixing the ingredients is to properly and closely and semi-permanently unite the formaldehyde solution with linseed oil. The proportions which have so far given best results are 1000 cubic centimeters of the formaldehyde solution, and 400 cubic centimeters of raw linseed oil. These two ingredients in the proportions named are first mixed in a "homogenizing apparatus" as described and illustrated in the patent to Otto Nielsen, Number 1,654,268, patented December 27, 1927. This mixing apparatus and process resulting in a very close and more or less permanent joinder of these two usually-unmixable ingredients.

This formaldehyde-oil homogenization is strained, and then dissolved with about 1000 grams of resorcinol and then, with reasonable celerity, brought up to a temperature of 30° centigrade approximately.

A solution is next made by dissolving some 10 grams of sodium hydroxide in 50 to 75 cubic centimeters of the 40% solution of formaldehyde, which is brought to boiling temperature, and cooled off to approximately 30° centigrade.

The formaldehyde-oil-resorcinol solution is brought from the mixing or homogenizing apparatus from its starting temperature of approximately 30° centigrade to a final temperature of about 80° centigrade very slowly, at the same time adding drop by drop, the sodium hydroxide formaldehyde solution.

The combined solution is then cooled off with considerable celerity, again to about 30° centigrade.

The varnish is now ready to be used.

- 8 The consistency of this varnish may be varied by going below or above the finishing temperature of 80° centigrade, also by the addition of softening or filling material, such as shellac, lampblack, or (and) china clay.
- 10 In use, the finishing temperature of 80° centigrade with its sudden cooling to 30° centigrade represents the correct temperature range when the pressing matrices are heated to a temperature of about 180° centigrade and 15 the record is pressed at a rate not exceeding 1 second for the pressing operation. Should these main conditions for pressing be varied, the temperatures would have to be varied to correspond so that the proper condition of the 20 varnish coating would apply for any new conditions of pressing.

During the operation of pressing the record, the linseed oil from the solution, which has been thoroughly but temporarily mixed 25 into the formaldehyde and the other ingredients, through the action of the homogenizing apparatus, is forced out of the solution and thoroughly impregnates the cardboard disk, thus automatically treating the 30 disk both to make it impervious to moisture and to carry with the oil certain of the other ingredients to thoroughly impregnate the disk material to furnish a complete joinder between the coating and the disk itself. This 35 results in a unified record structure free of the defects common to such laminated or built-up records, such as air bubbles, separation of the coating from its back stock, and the breaking of the needle through the coating into the 40 fibrous back stock.

A record of this type may be pressed in multiple in a high-speed press of the printing-press type from a continuous wide sheet of the fibrous or cardboard material, the individual records afterwards being cut from the sheet, thus assuring very rapid production 45 of the record. The coating material has been found to be very hard and durable and without excessive scratch on the surface when the record is being played. The coating is applied to the flexible cardboard sheet in a thickness slightly greater than the depth of the standard phonograph groove, which is about three thousandths of an inch.

55 It is to be understood that the present disclosure is for the purpose of illustration only, and that the invention is not limited thereto. To those skilled in the art, many modifications of the invention will be readily apparent, and it will also be obvious to such skilled persons that part of the concept may be used without other parts thereof, many such combinations of the parts readily suggesting themselves. Therefore, it should be, and is to be 65 distinctly understood that for a definition of

the limitations of the invention, reference must be had to the appended claims.

Having now described the invention, what is claimed as new and for which Letters Patent of the United States is desired is:

70 1. The process of compounding the ingredients for a sound record, comprising the steps of thoroughly mixing a formaldehyde solution and linseed oil, dissolving the resulting solution with resorcinol, mixing sodium hydroxide with a formaldehyde solution and applying the resulting mixture, drop by drop, to the former mixture, and then cooling the combination mixture from its mixing temperature of approximately 80° centigrade to 30° 75 centigrade.

75 2. The process of producing a heat and pressure hardening condensation product comprising making a solution of a vegetable oil, formaldehyde, and resorcinol; slowly adding a solution of sodium hydroxide and formaldehyde, and cooling the resulting liquid.

80 Signed at New York, in the county of New York and State of New York, this 5th day of October, A. D. 1927.

85 ADOLF HAWERLANDER.

85

100

105

110

115

120

125

130